

Sept. 8, 1942.

G. B. JONAS

2,295,082

PERMANENT MAGNET AND METHOD OF MAKING THE SAME

Filed June 29, 1939



INVENTOR  
G.B. JONAS

E. F. Wendoroth  
ATTORNEY

## UNITED STATES PATENT OFFICE

2,295,082

PERMANENT MAGNET AND METHOD OF  
MAKING THE SAME

Gottfried Bruno Jonas, Eindhoven, Netherlands,  
assignor, by means assignments, to Hartford  
National Bank and Trust Company, Hartford,  
Conn., as trustee

Application June 29, 1939, Serial No. 281,988  
In Germany December 6, 1938

21 Claims. (Cl. 175—21)

This invention relates to permanent magnets and to a method of manufacturing them.

The permanent magnet according to the invention exhibits the feature that it consists of a Ni-Al-Fe alloy having a cobalt content of 16 to 30%, a nickel content of 12 to 20% and an aluminium content of 6 to 11% and that in one (principal) direction (anisotropic) it has a  $(BH)_{max}$  value which is at least 2,000,000, for instance 4,000,000 to 5,000,000, and which is at least 50%, for instance 100 to 200%, higher than that of a permanent magnet which is made from the same alloy, but whose magnetic properties are at least substantially equal in all directions (isotropic). Since, as is well known, the size and weight of magnets are dependent upon the  $(BH)_{max}$  value of the magnet steel used, the advantageous results obtained by the present invention will be readily appreciated.

The magnets according to the invention preferably have a cobalt content of about 20% to 25%, a nickel content of about 13% to 17% and an aluminum content of about 7% to 10%, and with such compositions it is possible to obtain  $(BH)_{max}$  values greater than 3,000,000. I have found that such high  $(BH)_{max}$  values are due to the pronounced arched shape of the demagnetization curves and, as is well known, the fullness factor

$$\frac{(BH)_{max}}{B_r \times H_c}$$

is decisive for this shape. Magnets according to the invention having a  $(BH)_{max}$  value of at least 3,000,000 have a fullness factor of at least 0.45, generally 0.50 or more.

The magnets according to the invention can be made by subjecting the alloys to the action of a magnetic field during the cooling required for magnetic hardening.

Figs. 1 and 2 are demagnetization curves of permanent magnets according to the invention.

It is already known that the magnetic properties of certain ferro-magnetic materials having a high permeability are greatly influenced when, during the thermal treatment, the cooling from high temperatures is effected in a magnetic field.

This effect has also been examined with alloys for permanent magnets (see periodical "Nature" dated July 30, 1938, page 209). This periodical refers to an iron alloy for permanent magnets of the Ni-Al type which consists of 18% Ni, 10% Al, 12% Co, 6% Cu and 54% Fe and is cooled from a temperature of 1200° C. in a magnetic

field. In this case an improvement in the remanence and in the  $(BH)_{max}$  value is obtained. The remanence, for instance, was raised from about 7350 to about 7900 Gauss and the  $(BH)_{max}$  from 1,500,000 to 1,800,000.

As a possible explanation of the influence of the magnetic field it is pointed out that when ferro-magnetic materials are not subjected to a magnetic field during the cooling operation, they show the same magnetic properties in all directions. When using a magnetic field during the cooling operation the material exhibits anisotropy in such manner that, after subsequent magnetisation in a direction corresponding to the direction of the magnetic field during cooling, the magnetic properties in this direction are improved whereas the magnetic properties in other directions are reduced.

It appears from the considerations stated in this respect in the above-mentioned periodical that the said process of cooling in a magnetic field yields an improvement of about 7% in remanence and of 20% in  $(BH)_{max}$  for magnet steel, but that surprising improvements are not to be expected in this field. This tallies with the prevailing theoretical conceptions and with the fact that most of the alloys used in practice do not show at all or only slightly show this effect.

I have found that treatment in a magnetic field yields quite unexpected results and more particularly permits one to obtain  $(BH)_{max}$  values up to about 5,000,000, when used for the alloys stated in the preamble. It is remarked in this respect that up until now it has been possible only in special cases to produce a permanent magnet having a  $(BH)_{max}$  value exceeding 2,000,000. None of the commercial magnets have such values, but have values ranging between about  $1.8 \times 10^6$  and  $1.9 \times 10^6$ .

The progress according to the invention is more surprising, because a group of Ni-Al-Fe alloys is used which is very uneconomical and hence unusual in practice viz. alloys having a high cobalt content (more than 16%), while at the same time I obtain permanent magnets affording maximum economy. The permanent magnets according to the invention must be magnetized subsequent to the cooling in the direction of the lines of magnet force used to magnetize the magnet during the cooling, i. e. the lines of force during the subsequent magnetization should substantially coincide with the magnetic lines of force used during the cooling. If the magnetic lines of force during the subsequent magnetization were perpendicular to the direction of the

lines of force used during the cooling, the high  $(BH)_{max}$  value of the present invention would not be obtained. When I refer to the improvement in  $(BH)_{max}$  value of a permanent magnet according to the invention, I mean the improvement over a permanent magnet of the same composition, but which is subjected to a magnetization only after the heat treatment. The magnetic field preferably has an intensity of more than 3,000 Gauss.

The cooling operation may be effected in a usual manner which is best suited for obtaining favorable magnetic and mechanical properties, and one skilled in the art can select that cooling method which is best suited for use with a certain type of alloy when the cooling is effected without the application of a magnetic field. I employ the same cooling methods when applying the magnetic field during the cooling.

Furthermore it has been found advisable that the action of the magnetic field should take place at least in a temperature-interval which extends from the Curie-temperature to about 150° C. below this temperature and which is a part of the temperature-interval traversed during the cooling of the alloy necessary for hardening. I have found, that the time during which the temperature of the alloy remains in this interval between the Curie-point and the temperature 150° C. below this point has an influence on the magnitude of the effect. From this it follows that the process is particularly suitable for alloys with which, during the cooling stage of the treatment hitherto used, the time during which the temperature of the alloy remains within this interval has a certain minimum duration, e. g. 30 seconds, for optimum magnetic properties. I have found that in these cases the average cooling speed in the usual cooling operation, say between 1,250° C. and 600° C., should be low, i. e. about 10° C. per sec. at the utmost, and preferably about 1° C. to 5° C. per sec. In connection with the internal change of the alloy necessary for the occurrence of the effect, during the action of the magnetic field, it is advantageous to use alloys having a high Curie-point, for instance higher than about 780° C. The above-described alloys containing more than 16% Co can satisfy this condition.

As regards the aluminium content it is to be remarked that this should be adapted by a judicious choice to the contents of the other elements, and primarily to the nickel content.

In order to obtain excellent results as regards the value of  $(BH)_{max}$  it is advisable that the nickel content should not exceed 17%.

The use of copper, which is desirable in many modern magnet-steel alloys, is not essential and a high content, i. e. above 7%, is even inadvisable. However, I have found that in obtaining extremely high  $(BH)_{max}$  values it is advisable to admit small quantities of copper, for instance 1 to 3%. Generally it is advisable to reduce the nickel content in the case of high copper contents.

Titanium, which has also proved to be such a valuable element for various magnetic steel alloys and was present in the best magnetic steels hitherto known, is not an essential element of my alloy, although a total percentage of Al and Ti of less than about 12%, the Al percentage being from 6% to 11%, may be used in my alloy. However, a high titanium content, for instance more than about 5%, has proved to be detrimental.

In the following Table I are given several examples from which appears that the whole above-mentioned field of alloys can be split up into sections each of which shows particular magnetic properties.

Table I

| No. | L.                          | Percent                                     | Remanence<br>Br | Coercive<br>force | $(BH)_{max}$            |
|-----|-----------------------------|---------------------------------------------|-----------------|-------------------|-------------------------|
| 10  |                             |                                             |                 |                   |                         |
| a   | {Ni<br>Co<br>Al             | 14-20<br>21-25<br>8-10                      | 9,750-13,500    | 300-560           | 2-3.5×10 <sup>4</sup>   |
| b   | {Ni<br>Co<br>Al<br>Ti       | 14-18<br>22-25<br>6-8<br>0.4-4              | 9,200-12,000    | 470-765           | 2.5-4.2×10 <sup>4</sup> |
| c   | {Ni<br>Co<br>Al<br>Ti<br>Cu | 13-16.5<br>18.5-25<br>6.5-8.5<br>1-3<br>1-7 | 9,300-11,250    | 510-720           | 3-4×10 <sup>4</sup>     |
| d   | {Ni<br>Co<br>Al<br>Cu       | 12-15<br>20-27.5<br>8-8.5<br>1.5-6.5        | 9,250-12,500    | 520-630           | 3.5-4.8×10 <sup>4</sup> |

From this table, which is based on the results obtained from about 50 test-series, it clearly appears that the region of alloys designated by a is preferably to be used when value is attached to extremely high values of the remanence. The kind of alloys designated by b, which contains Ni, Al and Co and in addition Ti should be used if it is attempted to raise the coercive force to the highest possible extent. It is to be remarked that both in the case a and in the case b the  $(BH)_{max}$  obtained with the largest values of the remanence and of the coercive force respectively has at the same time the remarkable value of about  $3.5 \times 10^4$  and  $4.2 \times 10^4$  respectively.

The kind of alloy denoted by c, which in addition contains copper with respect to the last-mentioned alloy, may also be used for this purpose, and the alloy d (without titanium) permits more particularly maximum values and this jointly with remarkable values both for the remanence and for the coercive force.

A large number of elements other than those mentioned up till now may be added in considerable quantities as additional alloy constituents such that in each instance the stated improvement of at least 50% in  $(BH)_{max}$  is obtained. However, a distinction must be made between those metals which do not influence the anisotropy effect, but do affect the magnetic properties of the alloys and those other metals of the periodic system which are usually present in permanent magnets and which affect both the anisotropy effect and the magnetic properties of the alloys. As examples of the former metal I might mention, silicon, vanadium, antimony, tin and sulphur, and as examples of the latter metals I may mention chromium and manganese. More particularly, assume that a magnet of an Al-Fe-Ni-Co alloy when treated in the usual prior art manner has a  $(BH)_{max}$  value of 1,500,000 and when treated in the manner of the present invention has a  $(BH)_{max}$  value which, due to the anisotropy effect, is double, i. e. 3,000,000. If an element such as silicon, vanadium, antimony, tin and sulphur is added to this alloy and the alloy is treated in accordance with prior art methods, the  $(BH)_{max}$  value will decrease to a value between about 1,000,000 and 1,500,000. However, the anisotropy effect is not affected by the addition of these elements and if the alloy is treated in the manner of the present invention, a  $(BH)_{max}$  value of about 2,000,000,

i. e. approximately double the value obtained when using the prior art treatment, will be obtained.

If, instead of the above mentioned elements, an element such as chromium and manganese, is added to the alloy and the alloy is treated in a prior art manner, the  $(BH)_{max}$  value will be decreased to about 1,000,000 to 1,500,000 but when the alloy is treated by the method of the present invention the  $(BH)_{max}$  value will be decreased to about 1,400,000, i. e. to a value less than double the value obtained by the prior art treatment. Additions of other elements such as, for instance, calcium and to a lower degree tungsten may give rise to a slight but clearly perceptible increase in a characteristic magnetic value, for instance in remanence, but as a rule they tend to influence the other characteristic magnetic values. It will be understood that neither the anisotropy-effect nor the magnetic properties are materially influenced by the presence of slight quantities of other elements, for instance, in the form of impurities (i. e. in quantities of the order of some tenths of a per cent).

When making use of the invention one might expect that the highest attainable  $(BH)_{max}$  value would occur with alloys whose  $(BH)_{max}$  value is about 2,000,000 (which is practically the highest attainable value up till now) without cooling in a magnetic field. To my astonishment I have found, however, that with these alloys the aniso-

a high cobalt-content and which, when heat treated in a manner suitable for obtaining an optimum  $(BH)_{max}$  value, have a remanence of more than 10,000 Gauss, the improvement in the  $(BH)_{max}$  value due to the remarkably strong anisotropy-effect of the steel is considerable and that in general the remanence has a considerable influence in obtaining high  $(BH)_{max}$  values. In this manner I have found it possible to obtain the unprecedented  $(BH)_{max}$  value of more than  $2.5 \times 10^6$  and even more than  $4.5 \times 10^6$ , while at the same time securing a very high remanence, for instance, more than 12,000 Gauss. Thus, the present invention makes it possible to comply in a practical manner with the frequent desire to have a high  $(BH)_{max}$  together with a high remanence.

In contradistinction to what has been said in the above article in "Nature" with respect to the change in coercive force I have found that more particularly with alloys according to the invention showing the higher  $(BH)_{max}$  values, not only the remanence but also the coercive force, measured in a preferred direction is increased. The enormous increase in the  $(BH)_{max}$  value is partly to be ascribed thereto.

In the following Table II are stated, by way of example, various alloys, which have been cooled according to a usual heat treatment (third column) and in a magnetic field (fourth column).

Table II

| No. | Composition in per cent |     |    |     |     | Optimum $(BH)_{max}$ obtained by making use of a usual thermal treatment without magnetic field, after annealing |                |                | Results obtained by making use of a thermal treatment corresponding to that of the preceding column, but in accordance with the invention in a magnetic field, after annealing |                |                | Average cooling speed in the cooling region between about 1,200° to 600° C. | Improvement in $(BH)_{max}$ expressed in per cent | Fullness factor $(BH)_{max} / (B \times H_s)$ |
|-----|-------------------------|-----|----|-----|-----|------------------------------------------------------------------------------------------------------------------|----------------|----------------|--------------------------------------------------------------------------------------------------------------------------------------------------------------------------------|----------------|----------------|-----------------------------------------------------------------------------|---------------------------------------------------|-----------------------------------------------|
|     | Ni                      | Al  | Co | Cu  | Ti  | $(BH)_{max}$                                                                                                     | H <sub>c</sub> | B <sub>r</sub> | $(BH)_{max}$                                                                                                                                                                   | H <sub>s</sub> | B <sub>r</sub> |                                                                             |                                                   |                                               |
| 1   | 16.0                    | 8.5 | 23 |     |     | 1,220,000                                                                                                        | 348            | 9,050          | 3,450,000                                                                                                                                                                      | 492            | 12,650         | °C. p./sec.                                                                 | 183                                               | 0.55                                          |
| 2   | 13.5                    | 8   | 24 | 1.5 |     | 1,320,000                                                                                                        | 370            | 9,450          | 3,770,000                                                                                                                                                                      | 503            | 13,100         |                                                                             |                                                   |                                               |
| 3   | 13.5                    | 8   | 24 | 3   |     | 1,680,000                                                                                                        | 535            | 8,300          | 4,790,000                                                                                                                                                                      | 615            | 12,700         |                                                                             |                                                   |                                               |
| 4   | 16                      | 7.8 | 25 |     | 2.8 | 1,600,000                                                                                                        | 604            | 7,600          | 3,087,000                                                                                                                                                                      | 640            | 10,000         |                                                                             |                                                   |                                               |
| 5   | 14                      | 7.1 | 24 | 3   | 2.4 | 1,720,000                                                                                                        | 595            | 7,900          | 3,780,000                                                                                                                                                                      | 660            | 11,050         |                                                                             |                                                   |                                               |
| 6   | 14                      | 7.5 | 20 | 6.5 | 1.8 | 1,650,000                                                                                                        | 620            | 7,350          | 3,250,000                                                                                                                                                                      | 676            | 9,825          |                                                                             |                                                   |                                               |
| 7   | 16.5                    | 8.1 | 20 | 1.1 | 2.3 | 1,824,000                                                                                                        | 640            | 8,150          | 3,117,000                                                                                                                                                                      | 685            | 10,200         |                                                                             |                                                   |                                               |

tropy-effect which can be obtained when making use of the invention manifests itself to a small extent only or is not available at all, whereas in contradistinction thereto it has been found that it is with magnet steel alloys having comparatively much lower optimum  $(BH)_{max}$  values that this effect occurs to a remarkable extent so that these magnet steels, which are unusual as regards composition, permit final values of the  $(BH)_{max}$  far exceeding the values hitherto attainable by means of the best kinds of steel.

Without cooling in a magnetic field higher values of  $(BH)_{max}$  generally involved hitherto a lower remanence; for instance,  $(BH)_{max}$  values of about 2,000,000 could only be attained at comparatively low values of the remanence, for instance not more than 9,000 Gauss. This is due inter alia to the fact that the improvement in  $(BH)_{max}$  could only be obtained by raising the coercive force, which increase was obtained to a greater or less extent at the cost of the remanence.

I have found that with steel alloys which have

55 60 65 70 75 79 84 89 94 99 104 109 114 119 124 129 134 139 144 149 154 159 164 169 174 179 184 189 194 199 204 209 214 219 224 229 234 239 244 249 254 259 264 269 274 279 284 289 294 299 304 309 314 319 324 329 334 339 344 349 354 359 364 369 374 379 384 389 394 399 404 409 414 419 424 429 434 439 444 449 454 459 464 469 474 479 484 489 494 499 504 509 514 519 524 529 534 539 544 549 554 559 564 569 574 579 584 589 594 599 604 609 614 619 624 629 634 639 644 649 654 659 664 669 674 679 684 689 694 699 704 709 714 719 724 729 734 739 744 749 754 759 764 769 774 779 784 789 794 799 804 809 814 819 824 829 834 839 844 849 854 859 864 869 874 879 884 889 894 899 904 909 914 919 924 929 934 939 944 949 954 959 964 969 974 979 984 989 994 999 1004 1009 1014 1019 1024 1029 1034 1039 1044 1049 1054 1059 1064 1069 1074 1079 1084 1089 1094 1099 1104 1109 1114 1119 1124 1129 1134 1139 1144 1149 1154 1159 1164 1169 1174 1179 1184 1189 1194 1199 1204 1209 1214 1219 1224 1229 1234 1239 1244 1249 1254 1259 1264 1269 1274 1279 1284 1289 1294 1299 1304 1309 1314 1319 1324 1329 1334 1339 1344 1349 1354 1359 1364 1369 1374 1379 1384 1389 1394 1399 1404 1409 1414 1419 1424 1429 1434 1439 1444 1449 1454 1459 1464 1469 1474 1479 1484 1489 1494 1499 1504 1509 1514 1519 1524 1529 1534 1539 1544 1549 1554 1559 1564 1569 1574 1579 1584 1589 1594 1599 1604 1609 1614 1619 1624 1629 1634 1639 1644 1649 1654 1659 1664 1669 1674 1679 1684 1689 1694 1699 1704 1709 1714 1719 1724 1729 1734 1739 1744 1749 1754 1759 1764 1769 1774 1779 1784 1789 1794 1799 1804 1809 1814 1819 1824 1829 1834 1839 1844 1849 1854 1859 1864 1869 1874 1879 1884 1889 1894 1899 1904 1909 1914 1919 1924 1929 1934 1939 1944 1949 1954 1959 1964 1969 1974 1979 1984 1989 1994 1999 2004 2009 2014 2019 2024 2029 2034 2039 2044 2049 2054 2059 2064 2069 2074 2079 2084 2089 2094 2099 2104 2109 2114 2119 2124 2129 2134 2139 2144 2149 2154 2159 2164 2169 2174 2179 2184 2189 2194 2199 2204 2209 2214 2219 2224 2229 2234 2239 2244 2249 2254 2259 2264 2269 2274 2279 2284 2289 2294 2299 2304 2309 2314 2319 2324 2329 2334 2339 2344 2349 2354 2359 2364 2369 2374 2379 2384 2389 2394 2399 2404 2409 2414 2419 2424 2429 2434 2439 2444 2449 2454 2459 2464 2469 2474 2479 2484 2489 2494 2499 2504 2509 2514 2519 2524 2529 2534 2539 2544 2549 2554 2559 2564 2569 2574 2579 2584 2589 2594 2599 2604 2609 2614 2619 2624 2629 2634 2639 2644 2649 2654 2659 2664 2669 2674 2679 2684 2689 2694 2699 2704 2709 2714 2719 2724 2729 2734 2739 2744 2749 2754 2759 2764 2769 2774 2779 2784 2789 2794 2799 2804 2809 2814 2819 2824 2829 2834 2839 2844 2849 2854 2859 2864 2869 2874 2879 2884 2889 2894 2899 2904 2909 2914 2919 2924 2929 2934 2939 2944 2949 2954 2959 2964 2969 2974 2979 2984 2989 2994 2999 3004 3009 3014 3019 3024 3029 3034 3039 3044 3049 3054 3059 3064 3069 3074 3079 3084 3089 3094 3099 3104 3109 3114 3119 3124 3129 3134 3139 3144 3149 3154 3159 3164 3169 3174 3179 3184 3189 3194 3199 3204 3209 3214 3219 3224 3229 3234 3239 3244 3249 3254 3259 3264 3269 3274 3279 3284 3289 3294 3299 3304 3309 3314 3319 3324 3329 3334 3339 3344 3349 3354 3359 3364 3369 3374 3379 3384 3389 3394 3399 3404 3409 3414 3419 3424 3429 3434 3439 3444 3449 3454 3459 3464 3469 3474 3479 3484 3489 3494 3499 3504 3509 3514 3519 3524 3529 3534 3539 3544 3549 3554 3559 3564 3569 3574 3579 3584 3589 3594 3599 3604 3609 3614 3619 3624 3629 3634 3639 3644 3649 3654 3659 3664 3669 3674 3679 3684 3689 3694 3699 3704 3709 3714 3719 3724 3729 3734 3739 3744 3749 3754 3759 3764 3769 3774 3779 3784 3789 3794 3799 3804 3809 3814 3819 3824 3829 3834 3839 3844 3849 3854 3859 3864 3869 3874 3879 3884 3889 3894 3899 3904 3909 3914 3919 3924 3929 3934 3939 3944 3949 3954 3959 3964 3969 3974 3979 3984 3989 3994 3999 4004 4009 4014 4019 4024 4029 4034 4039 4044 4049 4054 4059 4064 4069 4074 4079 4084 4089 4094 4099 4104 4109 4114 4119 4124 4129 4134 4139 4144 4149 4154 4159 4164 4169 4174 4179 4184 4189 4194 4199 4204 4209 4214 4219 4224 4229 4234 4239 4244 4249 4254 4259 4264 4269 4274 4279 4284 4289 4294 4299 4304 4309 4314 4319 4324 4329 4334 4339 4344 4349 4354 4359 4364 4369 4374 4379 4384 4389 4394 4399 4404 4409 4414 4419 4424 4429 4434 4439 4444 4449 4454 4459 4464 4469 4474 4479 4484 4489 4494 4499 4504 4509 4514 4519 4524 4529 4534 4539 4544 4549 4554 4559 4564 4569 4574 4579 4584 4589 4594 4599 4604 4609 4614 4619 4624 4629 4634 4639 4644 4649 4654 4659 4664 4669 4674 4679 4684 4689 4694 4699 4704 4709 4714 4719 4724 4729 4734 4739 4744 4749 4754 4759 4764 4769 4774 4779 4784 4789 4794 4799 4804 4809 4814 4819 4824 4829 4834 4839 4844 4849 4854 4859 4864 4869 4874 4879 4884 4889 4894 4899 4904 4909 4914 4919 4924 4929 4934 4939 4944 4949 4954 4959 4964 4969 4974 4979 4984 4989 4994 4999 5004 5009 5014 5019 5024 5029 5034 5039 5044 5049 5054 5059 5064 5069 5074 5079 5084 5089 5094 5099 5104 5109 5114 5119 5124 5129 5134 5139 5144 5149 5154 5159 5164 5169 5174 5179 5184 5189 5194 5199 5204 5209 5214 5219 5224 5229 5234 5239 5244 5249 5254 5259 5264 5269 5274 5279 5284 5289 5294 5299 5304 5309 5314 5319 5324 5329 5334 5339 5344 5349 5354 5359 5364 5369 5374 5379 5384 5389 5394 5399 5404 5409 5414 5419 5424 5429 5434 5439 5444 5449 5454 5459 5464 5469 5474 5479 5484 5489 5494 5499 5504 5509 5514 5519 5524 5529 5534 5539 5544 5549 5554 5559 5564 5569 5574 5579 5584 5589 5594 5599 5604 5609 5614 5619 5624 5629 5634 5639 5644 5649 5654 5659 5664 5669 5674 5679 5684 5689 5694 5699 5704 5709 5714 5719 5724 5729 5734 5739 5744 5749 5754 5759 5764 5769 5774 5779 5784 5789 5794 5799 5804 5809 5814 5819 5824 5829 5834 5839 5844 5849 5854 5859 5864 5869 5874 5879 5884 5889 5894 5899 5904 5909 5914 5919 5924 5929 5934 5939 5944 5949 5954 5959 5964 5969 5974 5979 5984 5989 5994 5999 6004 6009 6014 6019 6024 6029 6034 6039 6044 6049 6054 6059 6064 6069 6074 6079 6084 6089 6094 6099 6104 6109 6114 6119 6124 6129 6134 6139 6144 6149 6154 6159 6164 6169 6174 6179 6184 6189 6194 6199 6204 6209 6214 6219 6224 6229 6234 6239 6244 6249 6254 6259 6264 6269 6274 6279 6284 6289 6294 6299 6304 6309 6314 6319 6324 6329 6334 6339 6344 6349 6354 6359 6364 6369 6374 6379 6384 6389 6394 6399 6404 6409 6414 6419 6424 6429 6434 6439 6444 6449 6454 6459 6464 6469 6474 6479 6484 6489 6494 6499 6504 6509 6514 6519 6524 6529 6534 6539 6544 6549 6554 6559 6564 6569 6574 6579 6584 6589 6594 6599 6604 6609 6614 6619 6624 6629 6634 6639 6644 6649 6654 6659 6664 6669 6674 6679 6684 6689 6694 6699 6704 6709 6714 6719 6724 6729 6734 6739 6744 6749 6754 6759 6764 6769 6774 6779 6784 6789 6794 6799 6804 6809 6814 6819 6824 6829 6834 6839 6844 6849 6854 6859 6864 6869 6874 6879 6884 6889 6894 6899 6904 6909 6914 6919 6924 6929 6934 6939 6944 6949 6954 6959 6964 6969 6974 6979 6984 6989 6994 6999 7004 7009 7014 7019 7024 7029 7034 7039 7044 7049 7054 7059 7064 7069 7074 7079 7084 7089 7094 7099 7104 7109 7114 7119 7124 7129 7134 7139 7144 7149 7154 7159 7164 7169 7174 7179 7184 7189 7194 7199 7204 7209 7214 7219 7224 7229 7234 7239 7244 7249 7254 7259 7264 7269 7274 7279 7284 7289 7294 7299 7304 7309 7314 7319 7324 7329 7334 7339 7344 7349 7354 7359 7364 7369 7374 7379 7384 7389 7394 7399 7404 7409 7414 7419 7424 7429 7434 7439 7444 7449 7454 7459 7464 7469 7474 7479 7484 7489 7494 7499 7504 7509 7514 7519 7524 7529 7534 7539 7544 7549 7554 7559 7564 7569 7574 7579 7584 7589 7594 7599 7604 7609 7614 7619 7624 7629 7634 7639 7644 7649 7654 7659 7664 7669 7674 7679 7684 7689 7694 7699 7704 7709 7714 7719 7724 7729 7734 7739 7744 7749 7754 7759 7764 7769 7774 7779 7784 7789 7794 7799 7804 7809 7814 7819 7824 7829 7834 7839 7844 7849 7854 7859 7864 7869 7874 7879 7884 7889 7894 7899 7904 7909 7914 7919 7924 7929 7934 7939 7944 7949 7954 7959 7964 7969 7974 7979 7984 7989 7994 7999 8004 8009 8014 8019 8024 8029 8034 8039 8044 8049 8054 8059 8064 8069 8074 8079 8084 8089 8094 8099 8104 8109 8114 8119 8124 8129 8134 8139 8144 8149 8154 8159 8164 8169 8174 8179 8184 8189 8194 8199 8204 8209 8214 8219 8224 8229 8234 8239 8244 8249 8254 8259 8264 8269 8274 8279 8284 8289 8294 8299 8304 8309 8314 83

correspond to a magnet steel according to the invention, whereas curves 3 and 4 correspond to the same steel treated according to the third column of the table. For comparison both figures represent in dotted lines the de-magnetisation curve of a known modern magnet steel having a very high  $(BH)_{max}$ . It appears from the figures that the high  $(BH)_{max}$  of the magnets according to the invention primarily results from a highly raised remanence and a more arched shape of the de-magnetisation curve, although the improvement of the coercive force with respect to the same steel cooled without magnetic field (compare curves 1 with 3 and 2 with 4) is also material.

For a proper understanding of the commercial importance of the present invention, it should be noted that the results given in the above tables are not limited to magnets of small dimensions or to testpieces.

I claim:

1. A permanent magnet consisting of a ferrous alloy containing about 16% to 30% cobalt, about 12% to 20% nickel, about 6% to 11% aluminum and the remainder principally iron, said magnet being magnetically-anisotropic and having a  $(BH)_{max}$  value in the principal direction at least about 50% higher than the  $(BH)_{max}$  value of a substantially magnetically-isotropic permanent magnet of the same alloy.

2. A permanent magnet consisting of a ferrous alloy containing about 20% to 25% cobalt, about 13% to 17% nickel, about 7% to 10% aluminum and the remainder principally iron, said magnet being magnetically-anisotropic and having a  $(BH)_{max}$  value in the principal direction which is at least 2,500,000 and is at least about 50% higher than the  $(BH)_{max}$  value of a substantially magnetically-isotropic permanent magnet of the same alloy.

3. A permanent magnet consisting of a ferrous alloy containing about 20 to 25% cobalt, about 13.5% to 16.5% nickel, about 7.1% to 8.5% aluminum and the remainder principally iron, said magnet being magnetically-anisotropic and having a  $(BH)_{max}$  value in the principal direction which is equal to at least about 3,000,000 and which is at least 50% greater than that of a substantially magnetically-isotropic permanent magnet of the same composition.

4. A permanent magnet consisting of a ferrous alloy containing about 21% to 25% cobalt, about 14% to 20% nickel, about 8% to 10% aluminum and the remainder principally iron, said magnet being magnetically-anisotropic and having a  $(BH)_{max}$  value in the principal direction which is at least 2,000,000 and which is at least 50% greater than that of a magnetically-isotropic permanent magnet of the same alloy, and a remanence of at least 8,000 Gausses.

5. A permanent magnet consisting of a ferrous alloy containing about 23% to 24% cobalt, about 13.5% to 16% nickel, about 7% to 8.5% aluminum and the remainder substantially iron, said magnet being magnetically-anisotropic and having a  $(BH)_{max}$  value in the principal direction of at least 3,000,000.

6. A permanent magnet consisting of a ferrous alloy containing about 16% to 30% cobalt, about 12% to 20% nickel, about 6% to 11% aluminum, the remainder being iron and at least one of the elements titanium in an amount less than about 5% and copper in an amount less than about 7%, said magnet being magnetically anisotropic and having a  $(BH)_{max}$  value in the principal di-

rection of at least about 50% higher than the  $(BH)_{max}$  value of a substantially magnetically-isotropic permanent magnet of the same alloy.

7. A permanent magnet consisting of a ferrous alloy containing about 20% to 25% cobalt, about 13.5% to 16.5% nickel, about 7.1% to 8.1% aluminum, the optional inclusion of one or both of the elements copper in an amount less than about 6.5% and titanium in an amount less than about 2.8% and the remainder iron, said magnet being magnetically-anisotropic and having a  $(BH)_{max}$  value in the principal direction which is at least 3,000,000 and which is at least 50% greater than that of a magnetically-isotropic permanent magnet of the same alloy, and a remanence of at least 8,000 Gausses.

8. A permanent magnet consisting of a ferrous alloy containing about 23% to 24% cobalt, about 13.5% to 16% nickel, about 7% to 8.5% aluminum, the remainder being iron and small quantities of at least one of the elements copper and titanium, said magnet being magnetically-anisotropic and having a  $(BH)_{max}$  value in the principal direction of at least 3,000,000.

9. A permanent magnet consisting of a ferrous alloy containing about 16% to 30% cobalt, about 12% to 20% nickel, about 6% to 11% aluminum, not more than 5% titanium and the remainder principally iron, the total aluminum-titanium content being not more than about 12%, said magnet being magnetically-anisotropic and having a  $(BH)_{max}$  value in the principal direction at least about 50% higher than the  $(BH)_{max}$  value of a substantially magnetically-isotropic permanent magnet of the same alloy.

10. A magnetically-anisotropic permanent magnet consisting of a ferrous alloy containing about 14% to 18% nickel, about 22% to 25% cobalt, about 6% to 8% aluminum, about 0.4% to 4% titanium and the remainder principally iron, said magnet having a coercive force of more than 450 Oersteds and a  $(BH)_{max}$  value which is greater than 2,500,000 and which is at least 50% greater than that of a substantially magnetically-isotropic permanent magnet of the same composition.

11. A magnetically-anisotropic permanent magnet consisting of a ferrous alloy containing about 14% to 18% nickel, about 22% to 25% cobalt, about 6% to 8% aluminum, about 0.4% to 4% titanium and the remainder principally iron, said magnet having a coercive force of more than 450 Oersteds and a  $(BH)_{max}$  value which is greater than 3,000,000 and which is at least 50% greater than that of a substantially magnetically-isotropic permanent magnet of the same composition.

12. A permanent magnet consisting of a ferrous alloy containing about 20 to 27.5% cobalt, about 12% to 15% nickel, about 8% to 8.5% aluminum, about 1.5% to 6.5% copper and the remainder principally iron, said magnet being magnetically-anisotropic and having a  $(BH)_{max}$  value in the principal direction which is equal to at least about 3,500,000 and which is at least 50% greater than that of a substantially magnetically-isotropic permanent magnet of the same composition.

13. A magnetically-anisotropic permanent magnet consisting of a ferrous alloy containing about 13% to 16.5% nickel, about 18.5% to 25% cobalt, about 6.5% to 8.5% aluminum, about 1% to 3% titanium, about 1% to 7% copper and the remainder principally iron, said magnet having a  $(BH)_{max}$  value which is greater than

3,000,000 and which is at least 50% greater than that of a substantially magnetically-isotropic permanent magnet of the same composition.

14. In the manufacture of a permanent magnet the steps of forming a body of a ferrous alloy containing about 16% to 30% cobalt, about 12% to 20% nickel, about 6% to 11% aluminum and the remainder principally iron, and subjecting the body to a magnetic field during the cooling operation required for magnetic hardening.

15. In the manufacture of a permanent magnet, the steps of forming a body of a ferrous alloy containing about 16% to 30% cobalt, about 12% to 20% nickel, about 6% to 11% aluminum, and the remainder principally iron, subjecting the body to a magnetic field during the cooling operation required for magnetic hardening to thereby make the alloy magnetically-anisotropic, and subsequently magnetizing the body in a direction corresponding to the direction of magnetization during cooling to thereby obtain a  $(BH)_{max}$  value at least 50% higher than that obtained with the same alloy without magnetization during the cooling.

16. In the manufacture of a permanent magnet, the steps of forming a body of a ferrous alloy having a Curie-temperature above about 780° C. and containing about 16% to 30% cobalt, about 12% to 20% nickel, about 6% to 11% aluminum and the remainder principally iron, subjecting the body to a magnetic field during the cooling operation required for magnetic hardening and while the alloy is at a temperature between its Curie-temperature and a temperature lying about 150° below the Curie-temperature to thereby make the alloy magnetically-anisotropic, and subsequently magnetizing the body in a direction corresponding to the direction of magnetization during cooling to thereby obtain a  $(BH)_{max}$  value at least 50% higher than that obtained with the same alloy without magnetization during the cooling.

17. In the manufacture of a permanent magnet, the steps of forming a body of a ferrous alloy containing about 20% to 25% cobalt, about 13% to 17% nickel, about 7% to 10% aluminum and the remainder principally iron, subjecting the body to a magnetic field during the cooling operation required for magnetic hardening to thereby make the alloy magnetically-anisotropic, and subsequently magnetizing the body in a direction corresponding to the direction of magnetization during cooling to thereby obtain a  $(BH)_{max}$  value at least 50% higher than that obtained with the same alloy without magnetization during the cooling.

18. In the manufacture of a permanent mag-

net, the steps of forming a body of a ferrous alloy containing about 20% to 25% cobalt, 13.5% to 16.5% nickel, 7.1% to 8.5% aluminum and the remainder principally iron, subjecting the body to magnetization during the cooling operation required for magnetic hardening, and subsequently magnetizing the body in a direction corresponding to the direction of magnetization during the cooling to thereby obtain a  $(BH)_{max}$  value which is greater than 3,000,000 and which is at least 50% greater than that of a substantially-isotropic permanent magnet of the same composition.

19. In the manufacture of a permanent magnet, the steps of forming a body of a ferrous alloy containing about 23% to 24% cobalt, about 13.5% to 16% nickel, about 7% to 8.5% aluminum and the remainder principally iron, subjecting the body to magnetization during the cooling operation required for magnetic hardening and subsequently magnetizing the body in a direction corresponding to the direction of magnetization during the cooling to thereby obtain a  $(BH)_{max}$  value greater than 3,000,000.

20. In the manufacture of a permanent magnet, the steps of forming a body of a ferrous alloy containing about 20% to 25% cobalt, about 13.5% to 16.5% nickel, about 7.1% to 8.5% aluminum, the optional inclusion of one or both of the elements copper in an amount less than about 6.5% and titanium in an amount less than about 2.8% and the remainder iron, cooling the body in a magnetic field from a temperature of about 1200° C. to a temperature of about 600° C. at a rate of between about 1 and 4.3 degrees centigrade per second to thereby make the alloy magnetically-anisotropic, and subsequently magnetizing the body in a direction corresponding to the direction of magnetization during cooling to thereby obtain a  $(BH)_{max}$  value at least 50% higher than that obtained with the same alloy without magnetization during the cooling.

21. In the manufacture of a permanent magnet, the steps of forming a body of a ferrous alloy containing about 23% to 24% cobalt, about 13.5% to 16% nickel, about 7% to 8.5% aluminum, the remainder being iron and small quantities of at least one of the elements copper and titanium, subjecting the body to magnetization during the cooling operation required for magnetic hardening and subsequently magnetizing the body in a direction corresponding to the direction of magnetization during the cooling to thereby obtain a  $(BH)_{max}$  value greater than 3,000,000.

GOTTFRIED BRUNO JONAS.